

# UNITED STATES PATENT OFFICE.

NIELS G. SÖRENSEN, OF STOCKHOLM, SWEDEN, ASSIGNOR TO AKTIE  
BOLAGET URDA, OF SAME PLACE.

## METHOD OF DYEING LEATHER BLACK.

SPECIFICATION forming part of Letters Patent No. 243,000, dated June 14, 1881.

Application filed October 26, 1880. (No specimens.) Patented in France October 11, 1880.

*To all whom it may concern:*

Be it known that I, NIELS GEORG SÖRENSEN, of Stockholm, in the Kingdom of Sweden, have invented a new and useful Method of 5 Dyeing Leather Black, of which the following is a specification.

My invention relates to an improved method of dyeing leather black, by means of which such operation is effected in a more convenient, cleanly, effectual, and durable manner than is the case when the ordinary methods are employed. The leather to which the said method of dyeing applies is such as has been tanned—that is to say, treated by or with and containing 15 tannic acid, or gallic acid, or any of those derivations or combinations of or with such analogous acids as turn black when acted on by compounds or preparations of vanadium. The 20 particular derivations or combinations of the said acids on which the compounds or preparations of vanadium have the desired effect, and also the nature of the said compounds or preparations which it is desirable to employ, are known to chemists. The dyeing can be 25 effected at any time after the leather has been tanned, as above referred to. The action of the vanadic compound or preparation—which is employed in solution—on the surface or body of the leather treated is to turn it black. (The 30 word “black” is not employed here in its strictly literal sense, but in its ordinary acceptation.)

It will be well understood that in order not to in any way injuriously affect the quality of 35 the leather it will be most advantageous to employ a neutral vanadic solution, and I have

successfully employed a neutral solution of vanadate of ammonia containing one per cent. of the latter salt. In order to bring out a full black color I have found that the moderate 40 use and application of heat is of beneficial influence.

The blackening of leather by vanadium compounds or preparations, as hereinbefore described, is especially advantageous in the treatment of manufactured articles, such as boots and shoes, as the risk of damaging the upper portions of the same is avoided, and in the case of ornamental stitching in saddlery-ware the leather is rendered black, while the said 50 stitching retains its proper color. It also allows of the operation to be performed without soiling the hands of the operator. Another advantage is that by the employment of vanadic compounds or preparations the color can 55 be made to penetrate deeper into the leather than is the case with the ordinary dyes used.

I claim—

As an improvement in the art of dyeing leather black, subjecting to the action of a vanadic compound or preparation leather previously tanned with a substance containing an acid or acids which turn black when acted on by compounds or preparations of vanadium, substantially as described.

In testimony whereof I have signed my name to this specification in the presence of two subscribing witnesses.

NIELS GEORG SÖRENSEN.

Witnesses:

C. J. A. DICK,  
ALFRED P. P. HAIGH.